

June 28, 1938.

D. ROBERTS

2,121,826

DOOR JAMB

Filed Oct. 2, 1935



Fig. 1



Fig. 2



Fig. 3



Fig. 4



Fig. 5



Fig. 6

INVENTOR.

Dudley Roberts

BY

*Samuel Petrolak*

ATTORNEY.

## UNITED STATES PATENT OFFICE

2,121,826

## DOOR JAMB

Dudley Roberts, New York, N. Y., assignor to Rubatex Products, Inc., New York, N. Y., a corporation of Delaware

Application October 2, 1935, Serial No. 43,133

2 Claims. (Cl. 20—69)

My invention relates to a novel construction of door jamb and process of making the same and, more particularly, relates to a novel, cell tight door jamb and its process of manufacture.

Door jams, especially those used along the edges of subway doors, are usually made of a rubber composition to provide the desired softness combined with a seal-like enclosure. Difficulties have been experienced with such rubber because, in obtaining sufficient softness of the rubber employed, ruggedness against mechanical tear and weather wear are sacrificed with the result that such door jams have a relatively short life.

In a co-pending application Serial No. 717,550, filed Mar. 27, 1934, of which I am a joint inventor, there is described a novel rubber composition (details of which will be given hereinafter) comprising a cellular rubber in which each of the minute cells containing gas at a high pressure are sealed. This sealed cellular rubber is relatively much softer than solid rubber, thus supplying one of the essential properties desired. Inasmuch as each cell is sealed from all other cells, it does not absorb water or moisture from the air and therefore is not so readily attacked by atmospheric conditions. Finally, it may be given considerably greater ruggedness than can be obtained with solid rubber approaching the softness of this rubber.

In employing sealed cellular rubber, however, the method of manufacture does not commercially permit the direct molding thereof into the shape of a door jamb.

Accordingly, an object of my invention is to provide a novel rubber door jamb and a novel method of manufacture of the same.

A further object of my invention is to provide a novel sealed cell rubber door jamb and its method of manufacture.

There are other objects of my invention which together with the foregoing will appear in the detailed description which is to follow in connection with the drawing, in which:

Figure 1 is a perspective view of the side of a car with sliding door, having secured to its edges my novel form of door jamb.

Figure 2 is a detail showing one form of my novel door jamb.

Figures 3 to 5 are modified forms of the door jamb.

Figure 6 shows one form of molded material used to make the door jamb of Figure 2.

In order to understand the invention, it is

first necessary to describe the rubber composition which I employ in carrying out my invention.

The ingredients entering into the product are mixed in approximately the following percentages by weight:

|                                                | Per cent |
|------------------------------------------------|----------|
| Washed first grade pale crepe or smoked rubber | 40-75    |
| Sulphur                                        | 6-30     |
| Light calcined magnesia                        | 3-5      |
| Ground gilsonite                               | 12       |
| Lower melting bituminous substances            | 12       |

The base ingredient of the product is the rubber which is preferably of a pale crepe grade #1, obtained in sheets about  $\frac{1}{8}$ " to  $\frac{1}{16}$ " x 10" x 20".

These sheets of rubber are passed through masticating mills consisting of two rollers rotating in opposite directions as in the case of meshing gears. One roller, however, rotates slightly faster than the other, so that the rubber fed between the rolls tends to rub on the surfaces of the different speed rolls and a nib is formed as shown at 11, Figure 2 of the copending application, S. N. 717,550, referred to above. The extent of this nib depends on the relative speeds of the rolls and the nib in turn determines how much of the two surfaces 12 and 13 of the rubber engage and are masticated by the respective rolls 14 and 15.

The rolls are steam heated to a temperature of approximately 150° F. as the rubber sheets are fed between them. The rubber is masticated or softened in this process, the individual sheets combining into a single mass of soft rubber, the degree of mastication depending on the spacing of the rolls, the temperature and the period of operation. I have found, however, that a mastication of one pound per minute at a roller temperature of 150° F. is sufficient for my purposes.

To this resulting soft rubber mass is now added an asphalt product or soft bitumin, such as suffron or mineral rubber. This asphalt is divided into fine particles and passed through a sixteen mesh sieve. While the rubber revolves on the masticating rolls, these particles of bitumin are shovelled on and are uniformly distributed over the rubber. The heat of the rubber melts the bitumen which penetrates into and is absorbed by the rubber.

The bitumin acts as a flux at low temperatures in the stage of partial vulcanization to be explained hereinafter. Any other low temperature flux may be substituted, i. e., a low melting hydrocarbon of the asphaltic group of a bituminous or waxy nature, having fluxing properties, such

as paraffin wax and stearic acid. During this stage the rubber has turned from a light to a dark color.

- Ground gilsonite, divided into even finer particles than bitumin and passed through a one hundred and sixty mesh sieve, is now sprinkled or shovelled on the rubber, still passing through the masticating rolls. Gilsonite is an asphalt like bitumin, but has a much higher melting point. 5 It will accordingly not be melted by the rubber, but will nevertheless penetrate into, impregnate and be absorbed by the soft spongy mass of rubber. Gilsonite functions as a flux in a high temperature stage to be described hereinafter, and 10 may accordingly be replaced by any suitable high temperature flux such as a high temperature asphalt. In using the expression "flux", it will be understood that I mean a substance acting to amalgamate or assist in the vulcanizing.
- 15 20 Summarizing the above, three stages have been described. In the first, the rolls were heated to a temperature of 150° F. while masticating or softening the rubber to combine the individual sheets into a single soft spongy mass. Assuming twenty-four pounds of rubber, twenty-four minutes may 25 ordinarily be required for this operation.

In the second stage, a low temperature flux is applied to the rubber as it continues to pass over the rolls, in the proportions given above, and this, 30 by reason of the heat, melts into and is absorbed by the rubber.

In the third stage, a high temperature flux is admixed with the rubber while it passes through the rolls, again in the proportions given above. 35 The second and third stages take fourteen minutes additional to the twenty-four minutes for mastication and result in a rubber impregnated with a high and low temperature hydrocarbon. The molecular structure of rubber is theoretically 40 described as normally being in the form of a spiral. This may be thought as giving to the rubber its elasticity and strength. During the working of the rubber described above, a disturbance of the molecular structure apparently occurs and 45 the rubber tends to lose its natural qualities.

It is essential to provide a rest period for the rubber at this stage of the operations to permit the rubber to restore itself to its original condition.

50 Accordingly, in the next or fourth stage, the rubber, now flat, soft and porous, is permitted to cool off and is left to rest for about twelve hours, preferably in a dark, dry room at a temperature of from 80° to 100° F. The longer the rest 55 period, the more the rubber regains its original condition, but I have found that twelve hours will ordinarily be sufficient to restore it to about its original condition.

Following this rest period, these slabs of rubber 60 are placed on rolls maintained at temperatures of from 120° to 130° F. As the rubber passes between the rolls, additional slabs are added, which ultimately combine into a soft mass of rubber. When the mass has been formed with adjacent 65 engaging surfaces adhering, sulphur and light calcined magnesia, in the proportions given above, are added as the rolls rotate. Sulphur is the vulcanizer and the light calcined magnesia is the rubber toughener. Any equivalent rubber 70 toughener, such as zinc oxide, may replace the calcined magnesia. For thorough absorption, the rolling is continued for a period of about twenty minutes.

The product is now removed from the rolls in 75 strips or slabs of about one-half inch in thickness

and two feet in length. The distorting effect of passing the rubber through the rolls is now again corrected by providing a second twenty-four hour rest period in a dark, warm, dry room at about the same temperature as the previous rest period. 5 Again the length of the rest period may vary, but at least twenty-four hours is necessary and the longer this period, the more nearly the rubber is restored to normal.

The rubber is now placed on a warmer mill consisting of two rollers rotating at the same speed. The rubber is fed between the rolls maintained at a temperature of from 120° to 140° F. This is continued until the rubber again becomes soft and forms into a uniform plastic composite mass 15 and during which the rubber may be formed into slabs, boards, etc., after which a further rest period of twelve hours is provided. Or, if desired, the rubber may be passed through a forcing machine which I prefer to use for pre-forming the 20 rubber in any desired shape, such as aeroplane wings, struts, pontoons, etc. If preferred, the forcing operations may also be used to soften the rubber in the earlier roller stages described here- 25 before.

The various stages of treatment described above have resulted in agitating the rubber to such an extent that a quantity of air has been absorbed by the rubber. The presence of this air may have serious deteriorating effect during 30 the subsequent stages to be described hereinafter. This may be described as follows:

Like glass, rubber is a plastic or super-cooled viscous liquid. Normally, it would be crystalline, but is prevented from becoming so because of the 35 complexity of the molecules which are large and slow-moving due to the viscosity of the mixture. This super-cooled viscous liquid is chemically an unstable product which tends to stabilize itself. This is particularly true if the rubber is warmed 40 to just below melting point which favors crystallization. The presence of air under these conditions is particularly conducive to crystallization, a simple oxidation resulting from a relatively simple rubber compound which crystallizes out. 45

Moreover, rubber oxidizes easily because it has unsaturations or double bonds which tend to readily combine with the oxygen, especially under the influence of heat and pressure, thus making the rubber brittle. In the presence of air, rubber therefore tends to oxidize. Attacked or oxidized by even a small amount of air, the rubber becomes 50 brittle, as is well known.

To prevent this, the rubber, as is commonly known, is vulcanized, i. e., stabilized. This consists in heating the rubber with sulphur to form a vulcanized or stable product so that it no longer tends to combine with oxygen in the air. The sulphur forms a mixture of complex compounds which prevents crystallization and oxida- 55 tion.

The presence, however, of even a small quantity of air may result in an oxidation, for the reasons explained above, even before vulcanization sets in.

Accordingly, it is important to force out all 60 the air that may have mixed with the rubber before the stage of partial vulcanization, to be described, occurs.

To this end the rubber is passed between successive calenders maintained at a temperature 65 of from 130° to 150° F. The calender mill comprises a series of rolls decreasingly spaced from each other in successive steps. In the first step, as shown in Figure 4 of the application S. N. 717,550, referred to above, the rolls are relatively 70 75

far apart, in the next stage, closer, etc. The rubber passing through the calenders forces all the trapped air out and is reduced in size. After the rubber passes the last rolls, a sheet of cloth 5 is applied thereto to close faults appearing in the rubber and to prevent the rubber from contracting. The cloth, having a limited expansion, keeps the stretch in rubber and maintains it a predetermined thickness.

10 The rubber is now cooled to room temperature and the cloth removed, leaving a sheet of untreated rubber. The product is now ready for the two final stages of vulcanization to be described. These vary somewhat for different products. Approximately ten such sheets of rubber 15 may be placed with metal sheets interposed between each sheet of rubber, and the whole placed in a metal container having an internal dimension slightly larger than the combined sheets. 20 A cover is then fastened into place on the container. A number of these containers are then placed into a gassing autoclave which is then closed and fastened down. The autoclave has previously been aired by passing steam through 25 the container and heating it to a temperature of from 180° to 212° F. to remove moisture.

A vacuum pump is then connected to an inlet of the container to extract the air until a vacuum of about five inches is obtained. The evacuation 30 is important for the reasons already pointed out hereinbefore. When the container has been evacuated, gas is admitted into the autoclave at a pressure of from 150 to 200 atmospheres. Any inert gas, preferably non-combustible, and having 35 no affinity for raw rubber, such as nitrogen (N<sub>2</sub>), ammonia (NH<sub>3</sub>), helium (He) may be used for this. Thus air would be disastrous, if used. Forcing air into raw rubber at several hundred atmospheres pressure and at or near vulcanizing 40 temperatures, would tend to oxidize the rubber very rapidly and before vulcanization set in, resulting in an undesirable product. Moreover, it would be dangerous practice, because a spark would cause a terrific explosion.

45 While the gas is being forced into the rubber, steam at eight pounds pressure is admitted to the steam chest. About thirty minutes are necessary for the container to reach a stable temperature, and thereafter the container is maintained 50 at the same temperature continuing to supply steam at about eight pounds pressure.

The conditions in this stage are critical and accordingly both the pressure of the gas and the temperature of the container must be correct. 55 The rubber, while exposed to the gas, is in a soft plastic state and therefore readily receives the gas. The eight pounds of steam in the steam jacket produce a temperature at which partial vulcanization proceeds to a substantially uniform 60 degree throughout the body of the rubber. This partial vulcanization functions to harden the rubber sufficiently so that it retains the gas forced into the rubber. At this time substantially little or no expansion of the rubber has taken place 65 due to its confinement within the container.

The autoclave is now permitted to cool off under atmospheric conditions and subsequently cold water is forced through the steam jacket until a temperature of 60°-70° F. is reached. 70 This permits the rubber now in semi-cured state to set.

Excess gas in the autoclave is now removed. The rubber being partially cured, will hold gas under pressure in its individual cells. The rubber 75 sheets are now removed from the containers with

the result that the pressure is removed and the gas in the cells immediately expands the rubber about four times.

This partially cured rubber is now placed in a mold suitably constructed to form the shape 5 shown in Figure 6.

As shown in Figure 6, the mold is of a shape to produce rubber symmetrical in shape comprising two end portions 20 and a central offset portion 11 forming shoulders 14 and 15 with one 10 of the edges of each end portion 20 and shoulders 12 and 13 with each of the opposite edges of portion 20.

The partially vulcanized rubber placed in the mold for producing this special shape of rubber 15 is now subjected to the final vulcanization. Each mold is placed in a mold of the desired dimensions. Each mold is placed between platens and saturated steam is applied at ninety-five pounds for about forty to forty-five minutes. This is 20 the final stage of the process of the curing and expansion. The rubber expands to the size of the molds and at the same time complete curing or vulcanization of the rubber is obtained. The steam is now turned off and the product permitted to cool. If desired, cooling may be hastened by applying cold water. The end product is an expanded cellular inert gas filled product weighing about five pounds per cubic foot.

This stage, during which the vulcanization is 30 completed, must take place within forty-eight hours after the completion of the partial expansion and vulcanization. Otherwise sufficient gas may escape from the partially vulcanized rubber so that there is a material loss in volume. 35

In the event that more than forty-eight hours elapse before the last stage of the process occurs, it is preferable to regrind the material and add it into the new dough in small percentages.

It is also possible, alternatively, in the event 40 that more than forty-eight hours is to elapse, to take care of this condition by carrying on the first stage to a further degree of vulcanization than originally contemplated by applying the steam for a longer period of time or at a higher 45 temperature than is obtained by eight pounds of steam.

In fact, I have found from experiments that the first stage can be carried on at from eight to sixteen pounds of steam, although better results 50 are obtained at the lower range. When the greater degree of vulcanization occurs, the material can be kept for a longer period than forty-eight hours without the gas diffusion.

The final product, depending upon the percentages of the various ingredients used is a soft light rubber of multitudinous minute sealed cells, each cell apparently containing gas at a high pressure.

The rubber in the form of Figure 6 is bent 60 about an imaginary center of the portions 14 until the faces or edges of portions 20 are in contact with each other. Strips of fabric 18 and 19 (Figure 2) of relatively stiff composition are vulcanized to the rubber along the upper edges 65 of portions 20, fitting against the shoulders 12 and 13 and having protruding end portions 31. These protruding portions may now be secured to the edge of a door 23 (Figure 2) or 24 (Figure 1) by any suitable means as rivets 22. The rubber, when thus secured forms a hollow space 17. 70

The advantages of this construction will now be obvious. Not only does this celltight rubber have a greater resistance to weathering and greater resistance to mechanical injury, but be- 75

cause of the minute sealed cells, it provides a greater cushioning effect than is attainable with ordinary rubber. Moreover, by the special mold, a single inexpensive piece is formed with a hollow space to further increase the cushioning effect.

In Figures 3 to 5, I have illustrated several of the many modifications my invention may undergo. Thus, I may, if preferred, vulcanize the fabric 26 to the bottom edge of the rubber after the two faces of sections 20 have been brought into opposed relation. Or I may obtain any desired arrangement or shape or number of spaces such as arch 27 and oval 28 in Figure 4 or the two shown at 29 and 30 in Figure 5. These shapes and their arrangements depend merely on the shape of the mold.

Moreover, although I have described for purposes of illustration, one process and formula for manufacturing the sealed cellular rubber, it will be understood that I may vary this in the light of the present acquired knowledge for manufacturing this rubber. Thus, I may use the formula and process described in the application of Peel et al., 26,164, filed June 12, 1935, or of the appli-

cation of Roberts et al., 21,380, filed May 14, 1935.

I do not intend to be limited by the specific formulae, process or mold construction here illustrated, but intend rather to cover door jambs constructed of a sealed cellular rubber in inexpensive single molds. It will be obvious that the usual electrical contactors are placed in the space 17 and operated when the rubber is compressed by the closing of the sliding door 24 of car 25.

I claim:

1. A door jamb comprising fabric securing means, soft closed cell gas expanded rubber positioned in adhesive contact with said fabric securing means, the soft closed cell gas expanded rubber constituting the working face of the door 15 jamb.

2. A door jamb comprising fabric securing means, soft closed cell gas expanded rubber positioned in adhesive contact with said fabric securing means, the fabric securing means extending 20 along only a portion of the contacting surface of the closed cell gas expanded rubber.

DUDLEY ROBERTS.